

## UNITED STATES PATENT OFFICE

MARKUS WERDER, OF FRIEDLINGEN-LEOPOLDSHOME IN BADEN, GERMANY

## PROCESS FOR LOADING OR IMPREGNATING SILK AND SILK-TISSUE

No Drawing. Application filed July 9, 1928, Serial No. 291,488, and in Germany May 2, 1928.

For the purpose of charging or loading silk and silk-tissues it is known to treat the same several times in succession with a solution containing chiefly stannic tetrachloride, 5 the so-called pink-bath, and subsequently with a solution containing mainly secondary phosphate of sodium or di-sodium phosphate.

Immediately upon having been treated with stannic tetra-chloride as above stated, 10 the material is subjected to a thorough and exhaustive washing and cleaning process. For the purpose of loading the material to any desired degree so as to produce a product which will show a predetermined or de- 15 sired increase in weight the above described process is correspondingly repeated. It is usual to finally subject the loaded material to a treatment with a solution of sulphate of aluminium or the like or with a solution of an 20 alkali silicate or even with both in succession.

This method is objectionable especially on account of the repeated treatments with solutions of tin-tetrachloride, a great part of which is washed in the washing water and 25 can only be recovered by very expansive processes. A further objection resides in the fact, that the exhaustive washing process, to which the material is subjected immediately after the treatment with tin-chloride-bath, 30 involves considerable cost.

The object of my invention is to remedy these defects. With this object in view I first treat the silk material with a solution of tin-tetrachloride as usual and immediately 35 thereupon, after having removed the excessive stannic chloride from the wet material by shaking or squeezing, I subject the latter to the action of an acid solution of ammonium phosphate, preferably mono-ammonium 40 phosphate.

In proceeding in this manner I surprisingly found that it is possible to attain in this way a comparatively high loading result or in other words to ensure any desired loading 45 effect by way of a less number of tin and phosphate treatments than hitherto required for obtaining the same effect. It will be seen that a marked economy of work, time and chemicals is secured thereby and besides that 50 a further considerable economical advantage

resides in the fact that the expensive recovery of tin salts from the washing water is dispensed with; another advantage of the invention lies in the fact that there is no necessity of employing protective colloids, which must 55 be used with the known methods. Separations or precipitations in the final product do not occur; gloss and all of the other valuable properties of the silk are fully preserved therein.

The concentration of the tin-bath is preferably between 24 and 30° Bé., while the acid phosphate bath or solution preferably contains 10 to 12 percent of mono-ammonium phosphate and may be applied in a cold state. 60

In connection with the improved process above outlined in general, the silk material is subjected to a subsequent treatment with di-sodium phosphate, which is known in itself, containing about 12 to 16 percent and 65 at a temperature of about 50 to 60° C.

If desired the method according to the present invention may be combined with any other known loading methods. The di-sodium-phosphate may be replaced by soda just in accordance with the loading degree desired to be attained in the final product and it goes without mentioning that the method may be combined with the usual final step of treating the product with waterglass or even with a solution or bath of sulphate of aluminium previous to such waterglass treatment. 75

I shall now proceed to describe the successive step of my invention more in detail by way of a few specific examples.

*Example 1.*—A tintetrachloride-bath of 28° Bé.,

Shaking or squeezing of the material,

A cold mono-ammonium phosphate bath containing 12 percent of mono-ammonium phosphate and 1 percent of phosphoric acid,

A di-sodium-phosphate bath containing 15 percent of di-sodium phosphate and heated 95 to a temperature of 60° C.,

Simple washing and shaking of the treated material under treatment.

*Example 2.*—A tintetrachloride-bath of 24° Bé.,

Shaking or squeezing of the material under treatment,

A cold bath containing 12 percent mono-ammonium phosphate,

5 A di-sodium phosphate-bath containing 15 percent of di-sodium phosphate and heated to a temperature of 60° C.,

Washing and shaking of the treated material.

10 *Example 3.*—The steps as in Example 1 or Example 2 and subsequently

A bath of waterglass of the usual concentration of about 50° Bé.,

Washing and shaking, soaping, dyeing.

15 A loading effect of 30-40% is obtained by this treatment. If it is desired to have a loading effect, for instance, of 85 to 95% the described treatments must be repeated three times.

20 What I claim is:

1. A process of impregnating silk and silk-tissues with chemical substances for the purpose of increasing the weight thereof, consisting in first treating the material in the usual manner with a tinchloride solution and immediately thereafter with an acid solution of ammonium phosphate.

25 2. A process of impregnating silk and silk-tissues with chemical substances for the purpose of increasing the weight thereof, consisting in first applying the usual treatment with a tinchloride solution and immediately thereafter treating the material with a solution of mono-ammonium phosphate.

30 3. A process of impregnating silk and silk-tissues with chemical substances for the purpose of increasing the weight thereof consisting in first treating the material with the usual tinchloride-bath and thereupon treating the material with an acid solution of ammonium phosphate and finally removing excessive liquid therefrom.

35 4. A process of treating silk and silk-tissues with chemical substances for the purpose of increasing the weight thereof which comprises first treating the silk material with a solution of stannic chloride, then removing excessive liquid therefrom by shaking and squeezing, thereupon treating the still wet material with an acid solution of ammonium phosphate and finally treating the same with a solution of di-sodium-phosphate.

In testimony whereof I affix my signature.

DR. MARKUS WERDER.